

(No Model.)

L. HAAS.

BUILDING WALL COMPOUND.

No. 293,010.

Patented Feb. 5, 1884.



WITNESSES

W. E. Bowen  
Geo. H. Hanby

INVENTOR

L. Haas  
By Myself  
Attorney

# UNITED STATES PATENT OFFICE.

LEVI HAAS, OF CHESTER, PENNSYLVANIA.

## BUILDING-WALL COMPOUND.

SPECIFICATION forming part of Letters Patent No. 293,010, dated February 5, 1884.

Application filed March 2, 1883. (No model.)

*To all whom it may concern:*

Be it known that I, LEVI HAAS, a citizen of the United States of America, residing at Chester, in the county of Delaware and State 5 of Pennsylvania, have invented certain new and useful Improvements in Building-Wall Compounds, of which the following is a specification, reference being had therein to the accompanying drawings.

10 My invention relates to an improvement in building-wall compounds; and it consists in a process by which slag (the dross of furnaces) is employed as a substitute for stone and brick, and in the process of forming fragmentary 15 slag into suitable blocks for this purpose, and in the molds A, substantially as hereinafter more fully described.

In carrying out my invention I take three 20 parts of the slag of furnaces and one part of mortar, the mortar being made of one part lime and three and one-half parts of sand and one and one-half part of water, and this mortar I combine in a suitable proportion to permeate the mass with a cementing-mortar made 25 of one pint of alkaline solution of flint, ten pints of sand, one pint of clay, and one pint of powdered flint. I then take this mass and cast it into rectangular or cubical blocks by placing it into suitably-constructed molds. 30 The blocks are then removed from the molds and dried. The materials thus combined produce a very hard and valuable building material at little cost.

In the drawings, Figure 1 is a plan view, 35 and Figs. 2 and 3 are detail views.

The mold A is rectangular, and adapted for molding the compound into blocks or bricks.

The lateral wall B of the mold is rigidly secured to the bottom C, and has adjustably affixed thereto the longitudinal sides D and 40 D' by means of the hinges E E. The lateral end F is hinged to the longitudinal wall D, and has secured therein the staple h, which projects through the slot of hinged hasp G, secured to the longitudinal wall D', the parts 45 being held together by pin P, as shown.

The partitions H and h' are removably inserted into grooves formed in the bottom of the mold, and the longitudinal partitions h' are recessed at a, to receive the transverse partitions H, in order that the partitions may be readily displaced in removing the molded blocks; and to this end the walls B, D, D', and F are hinged together and secured by the hinged hasps G. 55

What I claim, and desire to secure by Letters Patent, is—

1. A building material composed of three parts of furnace-slag and one part of mortar made of lime, sand, and water, and combined 60 in suitable proportions with an additional cementing-mortar made of powdered flint, alkaline solution of flint, sand, and clay, substantially as described.

2. The combination of the mold-bottom C, 65 partitions H and h', walls B, D, D', and F, and hinged hasp G, substantially as shown, and for the purpose described.

In testimony whereof I affix my signature in presence of two witnesses.

LEVI HAAS.

Witnesses:

J. WALTER LINDSAY,  
H. A. CLOUD.